

Patented Sept. 26, 1933

1,928,453

# UNITED STATES PATENT OFFICE

1,928,453

## CEMENTED TANTALUM CARBIDE

Floyd C. Kelley, Schenectady, N. Y., assignor to  
General Electric Company, a corporation of  
New York

No Drawing. Application November 1, 1930  
Serial No. 492,872

3 Claims. (Cl. 75—1)

The present invention relates to sintered metal compositions generally known as cemented carbides. A composition of this general character is disclosed in Schreter reissue Patent No. 17,624 and consists of a carbide of an element of the sixth group of Mendelejeff's table of elements of the periodic system, for example tungsten carbide, and a metal of the iron group, for example cobalt, the latter constituting from about 3% to about 20% of the composition and acting as a cementing or binder medium for tungsten carbide particles in the composition.

It is one of the objects of the present invention to provide a hard, tough, cemented carbide cutting tool which may be shaped or ground easily and supplied with a keen cutting edge by means of ordinary emery grinding wheels. Other objects of the invention will appear hereinafter.

The present description will be limited to specific elements, a particular composition, and to details of procedure but with the understanding that any of these may be varied so long as the same or approximately the same results are attained.

25 In carrying out the invention, I employ tantalum carbide as the main constituent of the cemented carbide, the binder or cementing medium consisting of cobalt and aluminum. In my copending application Serial No. 478,557, filed 30 August 28, 1930, and of which the present application is a continuation-in-part, I have disclosed a composition consisting of tantalum carbide and a metal of the iron group. Although cobalt may be employed alone as a binder element for tantalum carbide, I have found that when the cobalt is mixed with an appreciable quantity of another metal, for example aluminum, and the mixture of cobalt and aluminum employed as a binder for tantalum carbide, the physical qualities of the composition may be considerably improved.

The tantalum carbide is prepared by adding about 12 grams of carbon, for example gas coke, to about 181.5 grams of tantalum, and milling 45 the tantalum and carbon together for about five hours. The milling produces a very intimate mixture of the materials which are then fired at a temperature varying from about 1550° to 1600° C. for about eight hours in a closed graphite tube and in hydrogen furnace. A similar carburizing process is disclosed in my copending application Serial No. 308,565, filed September 26, 1928.

55 The carbide thus formed is golden brown in color and is milled to break it up into a fine powder capable of passing through a 250 mesh screen. It is then mixed with a suitable quantity of binder material, for example with about 13% of a mixture of cobalt and aluminum the binder 60 consisting of about 90 parts by weight of cobalt

with 10 parts by weight of aluminum and pressed into my desired shape in a hydraulic press. The cobalt and aluminum binder is a eutectic composition having a melting point of about 1375° C.

The pressed material, usually in the form of a 65 tool bit, is sintered in a closed graphite tube in a hydrogen furnace at a temperature of about 1300° C. for about 1½ hours. If the cemented tantalum carbide bit thus formed is copper brazed to a steel shank, it is desirable to employ 70 a flux, for example borax, in the brazing operation, in order to secure a good joint between the shank and the bit.

Cemented tantalum carbide having the above 75 composition has a hardness of about 81 on the Rockwell A scale and a modulus of rupture of about 120,000 pounds per square inch, the latter figure being obtained on a tool bit as fired and without previous lapping.

Special grinding wheels, such as carborundum 80 wheels are not required to shape the tantalum carbide, since the latter may be shaped easily and quickly by grinding on an ordinary emery wheel. The cemented carbide may be given a very keen cutting edge which it is able to retain under severe 85 operating conditions.

What I claim as new and desire to secure by Letters Patent of the United States, is:

1. A hard, tough, sintered composition consisting substantially of tantalum carbide and a 90 binder material for said carbide, said binder material comprising from about 3% to about 20% of said composition, said binder consisting substantially of metal of the iron group and aluminum the aluminum comprising an appreciable 95 quantity but not more than about 10% of said binder.

2. A hard, tough, metal composition consisting substantially of tantalum carbide and a cementing medium therefor, said cementing 100 medium comprising from about 3% to about 20% of said composition and consisting of about 90 parts by weight of cobalt and about 10 parts by weight of aluminum.

3. A hard, tough, sintered composition consisting substantially of tantalum carbide and a binder material for said carbide, said binder material comprising from about 3% to about 20% of said composition, said binder consisting substantially of about 90 parts by weight of metal of the iron 110 group and about 10 parts by weight of aluminum.

FLOYD C. KELLEY.

115

120